

**1**

3,117,087

**METHOD OF MAKING GREASES**

Martin M. McCormick, Chicago, and Lewis D. Loring, Jr., Dolton, Ill., assignors, by mesne assignments, to Sinclair Research Inc., New York, N.Y., a corporation of Delaware  
No Drawing. Filed Sept. 28, 1960, Ser. No. 58,880  
6 Claims. (Cl. 252—41)

This invention relates to the manufacture of lubricating greases. More particularly, this invention relates to an improved process for the manufacture of greases thickened with lithium soaps of hydroxy fatty acids.

A conventional high temperature method employed in the manufacture of greases which are difficult to prepare in satisfactory smooth form such as greases thickened with lithium soaps of hydroxy fatty acids, includes shock cooling a hot grease mixture either statically or with agitation so that the melted soap crystallizes in the form of very fine particles. Recently, methods have been discovered which include cooling the grease mixture at a relatively low rate while employing various techniques for the avoidance or reduction of super cooling. However, these methods have been partially ineffective as a long-fibered grease is formed which has a strong tendency to agglomerate during the stirring or the agitation stages which are employed in these commercial methods. Furthermore, the agglomerates which are formed are not easily separated by milling the grease according to conventional procedures. This difficulty therefore results in a deterioration of product quality and poor yields.

In the processing of lithium-12-hydroxy stearate greases, normally dehydration temperatures in excess of 400° F. are employed in order to obtain maximum gelling effect of the soap thickener. When forming by known methods a lithium-12-hydroxy stearate grease using a maximum temperature of about 350° F., the resulting grease is a satisfactory product but yields, i.e., hardness for a given soap content, are less than obtained in the high temperature procedure. Due to the relatively high cost of the soap thickener, a grease having the highest yield or lowest soap content for a given consistency is highly desirable.

Thus the need for a process which gives a high-yield-low-soap content lithium grease which can be prepared in the conventional grease-making equipment capable of effecting a maximum temperature of about 300—350° F. is clearly evident. The process of this invention overcomes these above-mentioned problems and facilitates the manufacture of a high-quality lithium-12-hydroxy stearate grease using conventional steam kettle temperatures, i.e., a maximum of about 300 to 350° F. during dehydration.

The improved method of this invention includes heating in grease-forming proportions a mixture of an ester of 12-hydroxy stearic acid, a suitable mineral or petroleum lubricating oil and an aqueous solution of a soluble lithium neutralizing compound to form a grease composition using a maximum temperature of about 300 to 350° F. The lithium soap is formed in situ in all or a portion, for instance, at least about an equal part based on the soap-forming ester, of the mineral base oil and a more or less homogeneous liquid mixture of the soap, water and lubricating oil is treated until it is essentially dehydrated. The mixture is then cooled and a grease composition is obtained. The process of the present invention involves recycling the mixture at least during the initial dehydration phase, that is, while the temperature is in the range

**2**

from approximately 200 to 350° F., through a shearing device so that grease formed is turned over rapidly and subjected to shear. In accordance with the present invention, the recycling is conducted during the major portion or even essentially all of the period wherein the temperature is in the range of about 200 to 260° F. but can continue through the major portion or essentially all of the approximate 200 to 350° F. range. The initial dehydration period may include the soap-forming reaction.

- 10      Recycling to the shearing means only after the dehydration period, however, has been found to be ineffective in the low temperature (350° F. maximum) processes. Thus the recycling of the present invention should be from essentially the start of soap fiber formation (i.e., water removal causing soap crystallization). The period of dehydration ranging from about 200 to 260° F. is generally the time it takes for the water content of the grease constituents to drop from about 5 to 15%, e.g. about 10%, to a content of about 2 to 0.3% or less. This period can 15      be easily determined by measuring the water content of the recycle material. The rate of recycle should be that necessary to recycle the entire batch of grease constituents rapidly during the dehydration period. The rate of recycle is dependent on the rate of dehydration, temperature etc. but is generally a rate that gives at least about 0.02 batch turnover per minute, preferably at least about 0.1 batch turnover per minute. Some improvement in 20      yield is obtained when the batch turnover is less than .02 per minute. The rate can be as great as desired but little 25      30      if any reason has been found for exceeding a rate of about 1 batch turnover per minute.

The saponifiable materials employed in the production of the soaps of the present invention are the esters of 12-hydroxy stearic acid, preferably the lower alkyl, e.g., of up to about 8 carbon atoms, esters of 12-hydroxy stearic acid, such as the methyl ester or the glyceride. The saponifying agent used for the in situ formation of the soap may be any water-soluble lithium neutralizing compound as, for example, the inorganic oxides, hydroxides and carbonates of lithium. The neutralizing component provides essentially complete neutralization or conversion of the ester to the soap although some free ester or lithium base may remain. In the final grease the lithium 12-hydroxy stearate is provided in an amount sufficient to exert in the base oil the essential thickening action, and the soap will usually be about 5 to 15% of the grease composition and the major part of the total base-oil thickening component.

The oleaginous liquids employed in the greases produced by the method of this invention may be any suitable oils of lubricating characteristics, including the conventional mineral lubricating oils. Suitable mineral oils include those having viscosities in the range from about 100 to 2,000 seconds Saybolt Universal at 100° F., and may be either mixed, naphthenic or paraffinic in type, or blends thereof.

The greases may also contain various additives of the usual types such as corrosion inhibitors, oxidation inhibitors, antiwear agents, extreme pressure agents and so forth. Preferably, they contain an oxidation inhibitor, which may suitably be an oxidation inhibitor of the amine type, such as diphenylamine, phenyl alpha naphthylamine or tetramethyldiaminodiphenylmethane. Compounds of this type may be added either before or during the cooling down process. They are preferably added while the temperature of the grease is between about 300° F. and about 180° F.

In the process of this invention the mixture of the fatty constituents and the oil is usually raised to a temperature of about 190-220° F. to melt the fatty material before the addition of the lithium base. The steam is then turned on the kettle and the recycle is started to obtain a pressure of about 40 p.s.i.g., or more in the recycle line. Dehydration is then effected by raising the temperature to about 300° F. to 350° F., preferably, to about 320-350° F. During the period of dehydration, the batch of constituents are recycled under pressure around the kettle and through a restricted orifice-containing shearing device.

The shearing means employed is preferably of the type which gives a very effective shearing and dispersing action with only a small amount of kneading action, e.g., globe valve, colloidal mill etc. A particularly suitable device for this purpose is a shear valve, through which the grease mixture is passed with a substantial pressure drop into a confined passageway, so that a strong turbulence is set up in the fluid mixture. When the grease mixture is passed through such a valve with a sufficiently high pressure drop, the soap fibers are very effectively separated and dispersed without any material breaking or thickening such as occurs when the grease is subjected to substantial kneading action during cooling. The degree of dispersal of the fibers, and consequently the yield and product quality of the grease, is directly related to the pressure drop across the valve. For purposes of the present invention, the pressure drop across the shearing orifices can range from about 20 to 100 p.s.i.g., preferably about 50 to 80 p.s.i.g. Pressure drops of over 100 p.s.i.g. do not appear necessary although pressure drops up to about 200 p.s.i.g. or higher can be employed with no harmful effects to the final product. If desired, the grease composition may be further finished after dehydration by colloidial milling so as to obtain the desired grease consistency. Colloidal milling operations are subject to variance, depending upon the inlet temperature, mill size and the like. The colloid mill size or clearance is ordinarily from about .001 to .1 inch. Although in high temperature processes, recycling through the gear pump and open lines has been found sufficient, in the low tempera-

ture process of the present invention normally greater shear than that given by a conventional recycle gear pump alone is required for satisfactory yields.

The following example will serve to illustrate the method of preparing the greases of the present invention.

#### EXAMPLE I

2.4 lbs. of lithium hydroxide monohydrate were dissolved in 12 lbs. of water and then added at a temperature of about 200° F. to a mixture of melted fats and 120 lbs. of mineral lubricating oil. The melted fats comprised 1.5 lbs. of beef tallow and 13.5 lbs. of hydrogenated castor oil. The mineral oil had a gravity API of 23.2, viscosity SUS at 210° F. of 80.7, and a viscosity index of 62.5. The constituents were then heated and recycling was begun through a 1" globe valve with a pressure drop across the valve of 50 pounds per square inch and a recycle rate of 22.4 pounds per minute. When the temperature reached 210° F. the water content of the recycle material was 2.17%. The spongy appearance of the mixture had assumed subsided. When the temperature of the batch reached 260° F. recycling was stopped. The water content of the recycle material at this temperature was 0.42%. Heating was continued and when the temperature of the batch reached 306° F., recycle was resumed but with no pressure drop across the globe valve in order to dehydrate the material remaining in the recycle lines. When the temperature of the batch reached 326° F. the heating steam was turned off and finishing oil was added slowly. On reduction of the temperature to 255° F. 65 pounds of finishing oil had been added to the mixture. The kettle was allowed to sit until the temperature was reduced to 245° F. The product was then colloid milled at .005 clearance and the product was at 35 170° F.

#### EXAMPLE II

Several batches of lithium 12-hydroxy stearate greases 40 were prepared using substantially the same procedure and formulation as that of Example I and recycled around the grease kettle through different sized globe valves at vari-

Table I

| Recycle Line                                                     | 1" Valve | 1 1/4" Valve |       |       |       |       | 55<br>1 260 |
|------------------------------------------------------------------|----------|--------------|-------|-------|-------|-------|-------------|
|                                                                  |          | 315          | 320   | 315   | 320   | 322   |             |
| Pressure Drop, p.s.i.g.                                          | none     | 80           | 40    | 50    | 50    | 55    |             |
| Max. Temperature, ° F.                                           | 315      | 320          | 315   | 320   | 322   | 322   |             |
| Recycle Rate:<br>lbs./min.                                       | 30       | 30           | 4     | 16    | 31    | 22    |             |
| Charge turnover, min.                                            | 4.5      | 9            | 34    | 9     | 4     | 6     |             |
| No Recycle                                                       |          |              |       |       |       |       |             |
| Recycle Charge, lbs.:                                            |          |              |       |       |       |       |             |
| Beef Tallow                                                      | 1.5      | 1.5          | 3     | 1.5   | 1.5   | 1.5   | 1.5         |
| Hydrogenated Castor Oil                                          | 13.5     | 13.5         | 27    | 13.5  | 13.5  | 13.5  | 13.5        |
| Lithium Hydroxide Monohydrate                                    | 2.41     | 2.42         | 4.82  | 2.42  | 2.41  | 2.41  | 2.40        |
| Oil Blend                                                        | 120      | 120          | 240   | 120   | 120   | 120   | 120         |
| Finishing Oil Blend Addition, lbs.                               | 30       | 31           | 156   | 52    | 65    | 79    | 65          |
|                                                                  | 5169     | 5155         | 5130  | 5158  | 5165  | 5168  | 5195        |
| Sample No. 801:                                                  |          |              |       |       |       |       |             |
| Lithium Soap, wt. percent                                        | 9.00     | 9.00         | 7.00  | 8.00  | 7.50  | 7.00  | 7.50        |
| Oil Blend, wt. percent                                           | 90.85    | 90.89        | ----- | 91.87 | 92.41 | 92.88 | 92.41       |
| Moisture, wt. percent                                            | 0.07     | 0.04         | ----- | 0.04  | 0.01  | 0.05  | 0.08        |
| Free Li OH, wt. percent                                          | 0.08     | 0.07         | ----- | 0.09  | 0.08  | 0.07  | 0.01        |
| ASTM Penetrations:                                               |          |              |       |       |       |       |             |
| Unworked                                                         | 288      | 281          | 292   | 301   | 297   | 295   | 294         |
| Worked                                                           | 269      | 268          | 276   | 282   | 284   | 290   | 278         |
| 100,000-Regular                                                  | 300      | 304          | 312   | 309   | 313   | 314   | 308         |
| 100,000-Navy                                                     | 323      | 314          | 325   | 319   | 323   | 331   | 322         |
| 4 hour Shell Roll, 160 r.p.m. RT: ASTM Penetration Change        | +4       | -2           | +11   | +16   | +22   | +10   | -2          |
| 96 hour Shell Muller, 10 r.p.m. 150° F.: ASTM Penetration Change | +35      | +40          | +40   | +37   | +42   | +19   | +24         |
| MIL-G-10924A Pressure Bleed: percent separated oil               | 4.3      | 3.6          | 5.4   | 5.1   | 5.7   | 5.3   | 5.1         |
| Wheel Bearing 660 r.p.m. 250° F.: Leakage, grams                 | {        | Pass         | Pass  | Pass  | Pass  | Pass  | Pass        |
| ASTM Dropping Point, ° F.                                        | 0.9      | 1.6          | 1.6   | 2.0   | 1.0   | 1.8   | 1.9         |
|                                                                  | 384      | 382          | 383   | 381   | 382   | 382   | 384         |

<sup>1</sup> Recycle stopped at this point before complete dehydration at about 325° F.

ous pressure drops, maximum temperatures and recycle rates. For comparison, a run employing no recycling and no pressure drop across the valve is included. Except as indicated recycling was for essentially the entire dehydration period above about 200° F. The conditions and tests on the products are shown in Table I.

From the data of Table I it is evident that little improvement in yield, i.e., hardness for a given soap content, is obtained by recycle with no pressure drop when compared with no recycle at all. The data further show that the yield obtained from the process of the present invention, for instance as measured by the amount of finishing oil permitted for a product of given penetration, is significantly greater than that obtained from low temperature processing (maximum 330° F.) without recycle.

### EXAMPLE III

Employing the process of the present invention several batches of lithium 1-hydroxy stearate thickened greases of the same general formulation as Example I were prepared at 400 and 330° F. maximum dehydration temperatures by recycling the mixture during the entire dehydration period through a 1 inch globe valve. The constituents of the charge, recycle conditions and results are all shown in Table II.

Table II

|                                                                  | High Temp. (400° F.) |       |       |            | Low Temp. (330° F.) |       |
|------------------------------------------------------------------|----------------------|-------|-------|------------|---------------------|-------|
|                                                                  | 50                   | none  | none  | -----      | 80                  | none  |
| Recycle Pressure Drop, p.s.i.g.                                  | 50                   | none  | none  | -----      | 80                  | none  |
| Recycle Rate:                                                    |                      |       |       |            |                     |       |
| lbs./min.                                                        | 120                  | 33    | 4     | -----      | 30                  | 30    |
| Charge turnover, min.                                            | 1.25                 | 4.5   | 38    | -----      | 9                   | 4.5   |
| Recycle Charge, lbs.:                                            |                      |       |       | No Recycle |                     |       |
| Beef Tallow                                                      | 1.5                  | 1.5   | 1.5   | -----      | 3                   | 1.5   |
| Hydrogenated Castor Oil                                          | 13.5                 | 13.5  | 13.5  | -----      | 27                  | 13.5  |
| Lithium Hydroxide Monohydrate                                    | 2.43                 | 2.40  | 2.40  | -----      | 4.82                | 2.42  |
| Oil Blend                                                        | 135                  | 135   | 135   | -----      | 240                 | 120   |
| Finishing Oil Blend Addition, lbs.                               | 65                   | 65    | 65    | -----      | 155                 | 31    |
| Sample No. 801:                                                  | 5096                 | 5228  | 5243  | 5230       | 5130                | 5155  |
| Lithium Soap, wt. percent                                        | 7.00                 | 7.00  | 7.00  | 10.00      | 7.00                | 9.00  |
| Oil Blend, wt. percent                                           | 92.88                | 92.96 | 92.96 | 89.95      | -----               | 90.89 |
| Moisture, wt. percent                                            | 0.08                 | 0.02  | 0.01  | 0.03       | -----               | 0.04  |
| Free Li, OH, wt. percent                                         | 0.04                 | 0.02  | 0.03  | 0.02       | -----               | 0.07  |
| ASTM Penetrations:                                               |                      |       |       |            |                     |       |
| Unworked                                                         | 295                  | 294   | 294   | 340        | 292                 | 281   |
| Worked                                                           | 282                  | 285   | 286   | 338        | 276                 | 268   |
| 100,000—Regular                                                  | 315                  | 315   | 309   | 347        | 312                 | 304   |
| 100,000—Navy                                                     | 336                  | 332   | 330   | -----      | 325                 | 314   |
| 4 hour Shell Roll, 160 r.p.m. RT: ASTM Penetration Change        | +4                   | +11   | +2    | -----      | +11                 | -2    |
| 96 hour Shell Muller, 10 r.p.m. 150° F.: ASTM Penetration Change | -----                | +22   | +28   | -----      | +40                 | +40   |
| MIL-G-10924A Pressure Bleed: Percent separated oil               | 6.1                  | 5.9   | 5.1   | -----      | 5.4                 | 3.6   |
| Wheel Bearing 660 r.p.m. 250° F.: Leakage, grams                 | Pass                 | Pass  | Pass  | -----      | Pass                | Pass  |
| ASTM Dropping Point, ° F                                         | 385                  | 382   | 382   | -----      | 383                 | 382   |

The data of Table II demonstrate that low temperature recycle processing in accordance with the process of the present invention gave equally as good yield and product quality as high temperature recycle processing.

### EXAMPLE IV

A lithium grease was prepared from hydrogenated castor oil and 500 SUS viscosity at 100° F., 95 viscosity index mineral oil essentially as in Example I except that the grease mixture was not recycled under shear until a dehydration temperature of 330° F. was reached. Upon reaching a temperatures of 330° F., the grease mixture was recycled for 1 hour under 60 p.s.i.g. pressure drop across a 1" globe valve. For comparison a similar grease was prepared without recycling. The recycle rates, constituents and results are shown in Table III.

6  
Table III

|    | 5                                                                | Recycled for 1 Hour Under 60 p.s.i.g. Pressure Drop Across 1" Globe Valve After First Reaching 330° F. |       | No Recycle |
|----|------------------------------------------------------------------|--------------------------------------------------------------------------------------------------------|-------|------------|
|    |                                                                  | 120                                                                                                    | 120   |            |
| 10 | Charge Turnover, min.                                            | 1                                                                                                      | ----- | -----      |
|    |                                                                  | 5025                                                                                                   | 6038  | -----      |
| 15 | Sample No. 801:                                                  |                                                                                                        |       |            |
|    | Lithium Soap, wt. percent                                        | 12.50                                                                                                  | 12.40 | -----      |
|    | Mineral Oil, wt. percent                                         | 87.35                                                                                                  | 87.52 | -----      |
|    | Moisture, wt. percent                                            | 0.07                                                                                                   | 0.05  | -----      |
|    | Free LiOH, wt. percent                                           | 0.08                                                                                                   | 0.03  | -----      |
| 20 | ASTM Penetrations:                                               |                                                                                                        |       |            |
|    | Unworked                                                         | 277                                                                                                    | 298   | -----      |
|    | Worked                                                           | 283                                                                                                    | 285   | -----      |
|    | 100,000—Regular                                                  | 300                                                                                                    | 302   | -----      |
|    | 100,000—Navy                                                     | 302                                                                                                    | ----- | -----      |
| 25 | 4 Hour Shell Roll, 160 r.p.m. RT: ASTM Penetration Change        | +18                                                                                                    | -22   | -----      |
|    | 96 Hour Shell Muller, 10 r.p.m. 150° F.: ASTM Penetration Change | +12                                                                                                    | ----- | -----      |
|    | MIL-G-10924A Pressure Bleed: Percent Separated Oil               | 5.9                                                                                                    | 10.0  | -----      |
|    | Wheel Bearing 660 r.p.m. 250° F.: Leakage, grams                 | Pass                                                                                                   | Pass  | -----      |
|    | ASTM Dropping Point, ° F                                         | 0.2                                                                                                    | 1.9   | 396        |

Examination of Table III shows that the yield and quality of lithium 12-hydroxy-stearate greases made by recycling to the shearing means after reaching a temperature of 330° F., i.e., after the dehydration period, are essentially no better than those of the same type of grease made at the same maximum temperature without recycling.

We claim:

1. In a method for preparing a lubricating grease which includes heating in grease-forming proportions a mixture of an ester of 12-hydroxy stearic acid, a mineral oil of lubricating viscosity, and an aqueous solution of a lithium neutralizing compound to a temperature of about 300 to 350° F. until the mixture is essentially dehydrated, and cooling the mixture to provide a grease composition, the improvement which comprises recycling said mixture through a restricted shearing orifice during

the initial dehydration period and over the major portion of the dehydration period in the range of about 200 to 260° F., said recycling being effected with a pressure drop across said orifice of at least about 20 p.s.i.g. at a grease-forming mixture turnover rate of at least about .02 per minute and sufficient to increase the grease yield.

2. The method of claim 1 wherein the recycle is during initial dehydration and over the major portion of the dehydration period in the range of about 200 to 350° F.

3. The method of claim 1 wherein the batch turnover rate is at least about .1 per minute.

4. The method of claim 1 wherein the pressure drop across the shearing orifice is about 50 to 100 p.s.i.g. and the turnover rate is at least about 0.1 per minute.

5. The method of claim 4 wherein the ester is hydrogenated castor oil.

6. The method of claim 5 wherein the recycle is during initial dehydration and over the major portion of the dehydration period in the range of about 200 to 350° F.

References Cited in the file of this patent

UNITED STATES PATENTS

|    |           |                 |       |               |
|----|-----------|-----------------|-------|---------------|
| 10 | 2,542,159 | Stevens         | ----- | Feb. 20, 1951 |
|    | 2,704,363 | Armstrong       | ----- | Mar. 15, 1955 |
|    | 2,801,220 | Smith           | ----- | July 30, 1957 |
|    | 2,886,525 | Dilworth et al. | ----- | May 12, 1959  |
|    | 3,015,624 | Hencke et al.   | ----- | Jan. 2, 1962  |

UNITED STATES PATENT OFFICE  
CERTIFICATE OF CORRECTION

Patent No. 3,117,087

January 7, 1964

Martin M. McCormick et al.

It is hereby certified that error appears in the above numbered patent requiring correction and that the said Letters Patent should read as corrected below.

Column 5, line 20, for "1-hydroxy" read --- 12 hydroxy --; column 6, Table III, second column, line 13 thereof, for "+18" read ---18 ---.

Signed and sealed this 17th day of November 1964.

(SEAL)

Attest:

ERNEST W. SWIDER  
Attesting Officer

EDWARD J. BRENNER  
Commissioner of Patents